

Dec. 12, 1961

R. A. MOSHER ET AL

3,012,506

RESTRICTED AMMONIUM NITRATE PROPELLANT

Filed Jan. 3, 1958

*Fig. 1*



*Fig. 2*



INVENTORS

Robert A. Mosher  
Paul O. Marti, Jr.

*Michael Dufresne*  
ATTORNEY

# United States Patent Office

3,012,506

Patented Dec. 12, 1961

1

3,012,506  
RESTRICTED AMMONIUM NITRATE  
PROPELLANT

Robert A. Mosher and Paul O. Marti, Jr., Seymour,  
Ind., assignors to Standard Oil Company, Chicago,  
Ill., a corporation of Indiana

Filed Jan. 3, 1958, Ser. No. 707,066  
5 Claims. (Cl. 102—98)

This invention relates to solid propellants based on ammonium nitrate, which propellants are suitable for use in gas generators and rocketry.

A rocket motor and a gas generator have the common requirement namely, that the gas produced in the motor and the generator must be produced at a substantially uniform rate and uniform pressure. The pressure within the motor or gas generator may be determined within limits for the particular gas producing material by the gas exit orifice size or the valve portion. On the other hand the uniform rate of gas production is much more difficult to attain. In order to attain a substantially uniform rate of gas generation it is necessary to utilize a particular type of configuration for the gas generating composition and to control the burning area of the composition. Unless very special precautions are taken all surfaces of the gas generating composition present in the combustion zone will burn. In solid propellants even the narrowest of fissures will result in two burning surfaces, i.e. one on each side of the fissure. To illustrate a solid propellant composition in a cylindrical configuration cannot be fitted so tightly against the wall of the combustion chamber that burning of the cylinder surface is prevented, that is, in the absence of some special precaution a cylindrical grain would burn at both ends and the cylindrical surface.

A uniform rate of burning or a controlled change in rate of burning is attained by applying a relatively non-combustible coating to the surface of the propellant body where direct burning is to be prevented. This coating is commonly referred to as a restrictor or combustion restrictor. The requirements for satisfactory restrictors are stringent. In the first instance the restrictor must adhere to the surface of the solid propellant body. Also, the restrictor must be substantially non-porous; the presence of pores or holes in the coat results in combustion of the solid propellant at that point with resultant variation in the gas production rate. Also the restrictor must not develop fissures or cracks under prolonged storage conditions. It is an ordinary military requirement that solid propellants be able to withstand repeated changes of temperature from as much as  $-70^{\circ}$  F. to as much as  $+170^{\circ}$  F. without changing the gas production rate. Of course, it is understood that the restrictors must be relatively simple to apply to the surface to be prevented from burning and also relatively inexpensive.

An object of the invention is a restricted solid propellant grain using ammonium nitrate as the major gas producing material. Other objects will become apparent in the course of the detailed description.

FIGURE 1 shows one embodiment of the invention namely, a solid propellant body having a cylindrical configuration with a restrictor applied to the cylindrical surface.

FIGURE 2 shows a cross-section at 2—2 of FIGURE 1.

The gas generating solid propellant of the invention comprises a shaped body portion, formed of ammonium nitrate as the major component and an oxidizable binder therefor, and a combustion restrictor coat positioned immediately contiguous to that part of the surface of said body where direct burning is to be prevented, which restrictor consists essentially of the resin reaction product

2

of (a) an epoxy resin having an epoxide equivalent weight between about 165 and 215 derived from epichlorohydrin and a bisphenol with (b) a liquid polymeric polyamide reaction product of polyene fatty acids and an aliphatic polyamine, said polyamide having an amine number between about 250 and 350 and with (c) a polymethoxy acetal having the formula



where  $n$  is an integer having an average value between 3 and 10, said reactants having been present in said resin producing reaction mixture, in parts by weight per 100 parts of reaction mixture, as follows: said epoxy between about 50 and 25, said polyamide between about 15 and 65, and said acetal between about 35 and 10, and wherein said restrictor coat is obtained by contacting said surface with a mixture of said reactants.

The epoxy resin utilized in the restrictor coating of the instant propellant is derived from the reaction of epichlorohydrin and a bisphenol. The bisphenols utilized may be bi-phenol, a substituted bi-phenol, particularly those containing alkyl substituents having from 1 to 4 carbon atoms, or complex bi-phenol ethers or the more complex bisphenols having alkyl group joining the two phenyl groups. A particularly suitable bisphenol reactant is 2,2-bis-(*p*-hydroxyphenylpropane) which is commonly known as Bisphenol A. The particular epoxy resin produced from these reactants has an epoxide equivalent weight between about 165 and 215. The commercially available material derived from the reaction of epichlorohydrin and Bisphenol A and having an average epoxide equivalent weight of about 185 is particularly suitable. The term "epoxide equivalent weight" as used herein is in accord with the usage of Stivala in chapter 10 of "High Polymers" volume X, Schildknecht in Polymer Processes; Interscience Publishers Inc., 1956.

The liquid polymeric polyamide used as a reactant for the preparation of the resin reaction product is a reaction product of polyene fatty acids and aliphatic polyamines. This polyamide is one of the well known class of polymers whose method of preparation from polyene fatty acids and alkylene polyamines is described in U.S. 2,450,940. A particularly suitable class of polyamides is described in U.S. 2,705,223 at column 3. For the purposes of this invention the polyamides are liquid materials, i.e. materials which are liquid at temperatures below about  $100^{\circ}$  F. and preferably are liquid at ordinary atmospheric temperatures in the region of 30 to  $75^{\circ}$  F. In addition to being liquid materials the polyamides used in this invention have an amine number between about 165 and 215. The amine number is a measure of the free amine groups present in the polymer and is defined as the number of milligrams of potassium hydroxide equivalent to the free amine groups present in one gram of the polymer.

The third reactant present in the reaction mixture which produces the resin reaction product used as the restrictor is a polymethoxy acetal. The polymethoxy acetals have the formula:



The acetals which are suitable for use herein are those where  $n$  is an integer having an average value between 3 and 10. In general these acetals are available as mixtures of compounds and are sold on the basis of an average molecular weight as defined by the value of  $n$ . Those acetals wherein the average value of  $n$  is 4 or 5 are particularly suitable.

In order to have a restrictor coating meet the particular requirements it is necessary that the proportions of the

tree reactions be controlled. Based on 100 parts of rection mixture the parts by weight of each reactant pres-  
it is as follows: the defined epoxy reactant between  
about 50 and 25; the defined liquid polyamide be-  
tween about 15 and 65 and the defined acetal between  
about 35 and 10. To illustrate one end of the range of  
roportions contains said epoxy 50 parts, said polyamide  
5 parts and said acetal 35 parts. At the other end of  
the range the proportions are said epoxy 25 parts, said  
olyamide 65 parts and said acetal 10 parts. The amount  
of each reactant present may be varied between these  
imits as required by the particular use and by the particu-  
ir epoxy or polyamide or acetal used.

The solid propellant of the invention comprises a  
aped body portion formed of ammonium nitrate as the  
ajor component, and an oxidizable binder therefor. This  
ody portion may be any of the configurations commonly  
sed for gas generator purposes or rocket propulsion pur-  
oses. For example, a simple cylinder, a tube, a cylinder  
ositioned within a tube, various cruciforms, internal star  
aped openings with various types of external surfaces,  
rticularly cylindrical, etc. The restrictor is positioned  
mmediately contiguous to that part of the surface of  
he propellant body where direct burning is to be pre-  
ented. For example, in a tubular grain the annular ends  
ay be coated with a restrictor in order to force the burn-  
ing to be on the exterior and internal cylindrical surfaces  
nly. In another instance only a particular area of a  
ody portion may be coated with a restrictor to provide a  
ery short term control of burning area; for example, it  
ay be necessary to have all the surface burning but  
mmediately after ignition, pressure surges must be avoid-  
d and this is done by restricting only a small portion of  
he body to control burning for maybe  $\frac{1}{2}$  second and at  
e end of that time the restrictor coating will be re-  
oved by the combustion gases. Many methods of re-  
striction are known in this art and it is to be understood  
hat the solid propellant of the invention may assume any  
one of these shapes.

One embodiment of the invention is particularly de-  
cribed in the figures. In FIGURE 1 there is shown a  
olid propellant whose body portion 11 is a simple cylinder  
in shape. A restrictor coating 12 is applied to the  
ylindrical surface 13 of body portion 11. In this em-  
odiment the end surfaces 14 and 16 are not restricted.  
When placed in a rocket motor for example, as shown in  
FIGURE 2 U.S. 2,539,404 and ignited at surface 16 this  
rain will burn in cigarette fashion; the restrictor 12 will  
revent gases from igniting the cylindrical surface 13 of  
he body 11.

It can be seen by examination of the figures that the  
estrictor coating 12 must adhere tightly to surface 13 or  
ot gas would pass between the restrictor 12 and surface  
3 and cause surface 13 to burn beyond the perpendicular  
burning surface extending from 16. This type of burn-  
ing would tend to produce a conical shaped burning sur-  
ace which would result in progressively increasing  
amount of gas production rather than the desired uni-  
orm rate.

The thickness of the restrictor coating 11 will be de-  
termined by the particular requirements. In general non-  
porous restrictors are obtained in coats as thin as  $\frac{1}{64}$   
inch. It is usual to use a thicker restrictor coat and in  
general the coat will be between about  $\frac{1}{16}$  and  $\frac{1}{4}$  inch  
hick. It is to be understood that the restrictor coat should  
be no thicker than the requirements of the particular ap-  
plication since excess thickness of material results in un-  
economic costs.

Another embodiment of the solid propellant of the in-  
vention consists of a number of gas generating composi-  
tion pieces which are bonded into a unitary solid propel-  
ant by using the restrictor of the invention as a mortar  
between the individual gas generator composition pieces.  
For example, a large motor may require an amount of  
solid propellant of a size that cannot be produced in one  
piece. For example, a cigarette burning cylinder may be

too large to be handled in one piece. This cylinder may  
be prepared in 3 or 4 sections. These individual sec-  
tions may be formed into, in effect, a single cylinder by  
using the restrictor material as the adhesive between each  
5 section. To illustrate: a cylinder having a diameter of  
about 9 inches and about 20 inches long was sawed into  
four-quarters lengthwise. The four-quarters were then  
10 cemented into a cylinder using restrictor material and then  
the cylindrical surface was restricted as shown in FIG-  
URES 1 and 2. This compositing grain was burned in a  
rocket motor for a period of several minutes and burned  
at a constant pressure indicating that under this severe  
duty the restrictor coating completely prevented passage  
of gas and burning down the sides of the individual pieces.

15 The body portion of the solid propellant of the inven-  
tion consists essentially of ammonium nitrate as the major  
component and oxidizable binder or matrix forming ma-  
terial is also present to permit the ammonium nitrate to  
be formed into shaped configurations or grains.

20 The improved composition of the invention contains  
ammonium nitrate as the major component. The am-  
monium nitrate may be ordinary commercial ammonium  
nitrate such as is used for fertilizers. This commercial  
grade material contains a small amount of impurities and  
25 the particles are usually coated with moisture resisting ma-  
terial such as paraffin wax. Military grade ammonium  
nitrate which is almost chemically pure is particularly  
suitable. The ammonium nitrate is preferably in a finely  
divided particulate form which may be either produced  
30 by prilling or by grinding. The ammonium nitrate is the  
major component of the gas-generator composition and  
usually the composition will contain between about 65  
and 80% of ammonium nitrate.

35 In order to permit the shaping of the ammonium nitrate  
composition into definite configurations a matrix former  
or binder material is present. When ammonium nitrate  
decomposes free-oxygen is formed. Advantage of the  
existence of this free-oxygen is taken and oxidizable or-  
ganic materials are used as the binders. These oxidizable  
40 organic materials may contain only carbon and hydrogen,  
for example, high molecular weight hydrocarbons such as  
asphalts or residuums, and rubbers either natural or  
synthetic. Or, the oxidizable organic material may con-  
tain other elements in addition to carbon and hydrogen  
45 for example, Thiokol Rubber and Neoprene. The stoichi-  
ometry of the composition is improved, with respect to  
smoke production, by the use of oxygenated organic ma-  
terials as the binders. The binder or matrix former may  
be a single compound such as a rubber or asphalt or it  
50 may be a mixture of compounds. The mixtures are par-  
ticularly suitable when special characteristics are to be  
imparted to the grain which cannot be obtained by the  
use of a single compound.

55 The multi-component binder or matrix former com-  
monly consists of a polymeric base material and a plastic-  
izer therefor. Particularly suitable polymeric base ma-  
terials are cellulose esters of alkanoic acids containing from  
2 to 4 carbon atoms such as cellulose acetate, cellulose  
acetate butyrate and cellulose propionate; the polyvinyl  
60 resins such as polyvinylchloride and polyvinyl acetate are  
also good bases; styreneacrylonitrile is an example of a  
copolymer which forms a good base material. In gen-  
eral the binder contains between about 15 and 45% of  
the particular polymeric base material.

65 The plasticizer component of the binder is broadly de-  
fined as an oxygenated hydrocarbon. The hydrocarbon  
base may be aliphatic or aromatic or may contain both  
forms. The oxygen may be present in the plasticizer in  
ether linkage and/or hydroxyl group and/or carboxyl  
groups; also the oxygen may be present in inorganic sub-  
stituents particularly nitro groups. In general any plas-  
ticizer which is suitable for work with the defined poly-  
mers may be used in the invention. Exemplary classes  
70 of plasticizers which are suitable are set out below.

75 It is to be understood that these classes are illustrative

only and do not limit the types of oxygenated hydrocarbons which may be used to plasticize the polymer.

Di-lower alkyl-phthalates, e.g. dimethyl phthalate, dibutyl phthalate diethyl phthalate and dimethyl nitrophthalate. Nitrobenzenes, e.g. nitrobenzene, dinitrobenzene, nitrotoluene, dinitrotoluene, nitroxylene, and nitrodiphenyl. Nitrodiphenyl ethers, e.g. nitrodiphenyl ether and 2,4-dinitrodiphenyl ether.

Tri-lower alkyl-citrates, e.g. triethyl citrate, tributyl citrate and triamyl citrate.

Acyl tri-lower alkyl-citrates where the acyl group contains 2-4 carbon atoms, e.g. acetyl triethyl citrate and acetyl tributyl citrate.

Glycerol-lower alkanoates, e.g. monoacetin, triacetin, glycerol, tripropionate and glycerol tributyrate.

Lower alkylene-glycol-lower alkanoates wherein the glycol portion has a molecular weight below about 200, e.g. ethylene glycol diacetate, triethylene glycol dihexoate, triethylene glycol dioctoate, polyethylene glycol di-octoate, dipropylene glycol diacetate, nitromethyl propanediol diacetate, hydroxyethyl acetate and hydroxy propyl acetate (propylene glycol monoacetate).

Dinitrophenyl-lower alkyl-lower alkanoates, e.g. dinitrophenyl ethylacetate, and dinitrophenyl amyloctoate.

Lower alkylene-glycols wherein the molecular weight is below about 200, e.g. diethylene glycol, polyethylene glycol (200), and tetrapropylene glycol.

Lower alkylene-glycol oxalates, e.g. diethylene glycol oxalate and polyethylene glycol (200) oxalate.

Lower alkylene-glycol maleates, e.g. ethylene glycol maleate and bis(diethylene glycol monoethyl ether) maleate.

Lower alkylene-glycol diglycolates, e.g. ethylene glycol diglycolate and diethylene glycol diglycolate.

Miscellaneous diglycolates, e.g. dibutyl diglycolate, dimethylalkyl diglycolate and methylcarbitol diglycolate.

Lower alkyl-phthalyl-lower alkyl-glycolate, e.g. methyl phthalyl ethyl glycolate, ethyl phthalyl ethyl glycolate and butyl phthalyl butyl glycolate.

Di-lower alkyl-oxy-tetraglycol, e.g. dimethoxy tetra glycol and dibutoxy tetra glycol.

Nitrophenylether of lower alkylene glycols, e.g. dinitrophenyl ether of triethylene glycol and nitrophenyl ether of polypropylene glycol.

Nitrophenoxy alkanols wherein the alkanol portion is derived from a glycol having a molecular weight of not more than about 200. These may be pure compounds or admixed with major component bis(nitrophenoxy)-alkane.

A single plasticizer may be used or more usually two or more plasticizers may be used in conjunction. The particular requirements with respect to use will determine not only the polymer but also the particular plasticizer or combination of plasticizers which are used.

In addition to the basic components, i.e. ammonium nitrate binder and catalyst, the gas generator propellant composition may contain other materials. For example, materials may be present to improve low temperature ignitability, for instance oximes may be present or, asphalt may be present. Surfactants may be present in order to improve the coating of the nitrate with the binder and to improve the shape characteristics of the composition. Various burning rate promoters, which are not catalyst per se, may also be present.

The aromatic hydrocarbon amines are known to be gas evolution stabilization additives. Examples of these aromatic amines are toluene diamine, diphenyl amine, naphthalene diamine, and toluene triamine. In general the aromatic hydrocarbon amines are used in amounts between about 0.5 and 5 percent.

The mixture of ammonium nitrate, cellulose ester and oxygenated hydrocarbon is essentially as insensitive to shock as is ammonium nitrate itself. It is extremely difficult to get this particular mixture to burn. Smooth

burning is attained by the addition of a catalyst to the mixture. This catalyst is distinguished from the well known sensitizers. For example, nitro starch or nitro-glycerin may be added to ammonium nitrate in order to increase its sensitivity to shock and enable it to be more easily detonated for explosive use. Catalysts as a class do not promote sensitivity and are used to cause the ammonium nitrate composition to burn for example like a cigarette. The effectiveness of the catalyst is in general measured by its ability to impart a finite burning rate to a cylindrical strand of ammonium nitrate composition. The burning rate is specified as inches per second at a given pressure and temperature; usually these burning rates are obtained by a bomb procedure operating at 1000 p.s.i. and about 75° F. temperature.

Many catalysts which promote the burning of ammonium nitrate compositions are known. The inorganic chromium salts form the best known classes of catalysts. The better known members of this class are ammonium chromate, ammonium polychromate, the alkali metal chromates and polychromates, chromic oxide, chromic nitrate, and copper chromite. Ammonium dichromate is the most commonly used chromium salt. Various hydrocarbon amine chromates such as ethylene diamine chromate and piperidine chromate are also excellent chromium catalyst. Certain heavy metal cyanides particularly those of cobalt, copper, lead, nickel, silver and zinc are effective catalysts. The cyanamides of barium, copper, lead, mercury and silver are effective catalysts. The various Prussian blues are excellent catalysts.

In addition to the above primarily inorganic catalysts various organic catalysts are known. The organic catalysts are particularly useful when it is desired to have combustion products which are gases or vapors and thereby do not erode gas exit orifices. Two catalysts which do not contain any metal components are pyrogene blue (Color Index 956-961) and methylene blue. Particularly suitable catalysts are the alkali metal barbiturates. Finely divided carbon such as carbon black present in amounts of several percent is effective alone as a catalyst however, carbon is generally used in combination with another catalyst as a burning rate promoter.

#### Test

45 The propellant body portion to which the restrictor coatings were applied in this test was a cylinder about 9 inches in diameter and about 20 inches long. The restrictor coating which was applied to the cylindrical surface had a thickness of approximately  $\frac{1}{16}$  inch. The solid propellant grains were then placed into a rocket motor and fired using an orifice such that the internal pressure in the combustion chamber was about 800 p.s.i. The particular propellant composition gave a burning time of about 200 seconds. In all cases the grain was carefully inspected after having been subjected to thermal cycling tests over the temperature range -50° F. to +150° F. in order to detect restrictor cracking and spalling.

50 The body portion consisted of an ammonium nitrate composition as follows: cellulose acetate 12%, acetyl triethyl citrate 9%, 9% of a 2:1 mixture of dinitrophenoxoethanol and bis(dinitrophenoxo)ethane, carbon black 4%, toluene diamine 1%, sodium barbiturate catalyst 3% and ammonium nitrate 62%.

55 In this test the epoxy resin was a commercial material which had an epoxide equivalent weight of 179-194 and is produced by the reaction of epichlorohydrin and Bisphenol A. The liquid polymeric polyamide was a commercial material having an amine number in the range of 290-320 and averaging about 305; this material is commonly known as Versamid 125. The polymethoxy acetal used has an average *n* value of 4 and is available commercially as PMAC-5; this material is a condensation product of methylvinyl ether and methanol. In this test the reaction mixture consisted of 45 parts by weight of

ersamid 125, 35 parts by weight of epoxy and 20 parts weight of PMAC-5.

This particular mixture has a reaction time of about hours prior to setting to a semi-solid material. In about 1-24 hours, dependent on atmospheric temperature, the action mixture sets to a hard tough solid. Prior to this the body portion which was to be restricted had been placed within a shell enclosing the cylindrical surface and spaced about  $\frac{3}{16}$  inch from the surface. The mixture of reactants at room temperature of about 80° F. was then poured into the space between the cylindrical surface of the body portion and the shell. In general it is best to bring the reactants into contact with the surface to be restricted almost immediately after the final mixing of the reactants. However, there is an appreciable time before the initial setting of the reactants and some delay may be tolerated. It is observed that a fair temperature rise takes place during the setting of the resin reaction product. In this instant the solid propellant was permitted to set for 4 hours to allow for completion of the resin reaction. The shell was removed and the restrictor coating carefully inspected for bubbles and incomplete coverage of the surface. This procedure gives a complete coverage of the surface with a bubble free impervious resin coat. This solid propellant was subjected to the temperature cycling test required by military specifications and was then fired in a rocket motor. A very uniform pressure was maintained in the rocket motor for the duration of the firing indicating that the restrictor coat successfully prevented burning of the cylindrical surface of the grain.

Thus having described the invention, what is claimed is:

1. A solid propellant comprising a shaped body portion, formed of ammonium nitrate as the major component and an oxidizable binder therefor, and a combustion restrictor coat positioned immediately contiguous to that part of the surface of said body where direct burning is to be prevented, which restrictor consists essentially of the resin reaction product of (a) an epoxy resin having an epoxide equivalent weight between about 165 and 215

derived from epichlorohydrin and a bisphenol with (b) a liquid polymeric polyamide reaction product of polyene fatty acids and an aliphatic polyamine, said polyamide having an amine number between about 250 and 350 and with (c) a polymethoxy acetal having the formula



where  $n$  is an integer having an average value between 10 and 15, said reactants having been present in said resin producing reaction mixture, in parts by weight per 100 parts of reaction mixture, as follows: said epoxy between about 50 and 25, said polyamide between about 15 and 65, and said acetal between about 35 and 10, and wherein said restrictor coat is obtained by contacting said surface with a mixture of said reactants.

2. The propellant of claim 1 wherein said epoxy resin has an epoxide equivalent weight of about 185 derived from epichlorohydrin and Bisphenol A, said polyamide has an amine number of about 305 and said acetal is the defined polymethoxy acetal wherein  $n$  is 4.

3. The propellant of claim 2 wherein the weight ratio of epoxy to polyamide to acetal is about 35:45:20.

4. The propellant of claim 1 wherein said shaped body portion is a cylinder and said restrictor coat is positioned immediately contiguous to the cylindrical surface of said cylinder, said coat being between about  $\frac{1}{16}$  and  $\frac{1}{4}$  inch thick.

5. The propellant of claim 4 wherein said body portion consists essentially of ammonium nitrate as a major component, and ammonium nitrate combustion catalyst in an amount between about 1 and 8 weight percent and between about 10 and 40 weight percent of a binder consisting essentially of cellulose acetate and an oxygenated hydrocarbon plasticizer therefor.

No references cited.